

Aug. 29, 1972

M. FAULSTICH ET AL  
GLASSES FOR TEMPERATURE-STABLE ULTRASONIC DELAY LINES  
OF LOW DAMPING CHARACTERISTICS  
Filed June 22, 1970

3,687,697

FIG. 1



FIG. 2



FIG. 3



INVENTORS

MARGA FAULSTICH  
NORBERT NEUROTH

BY

Burgess, Dinklage + Sprung

ATTORNEYS.

## 1

3,687,697

### GLASSES FOR TEMPERATURE-STABLE ULTRASONIC DELAY LINES OF LOW DAMPING CHARACTERISTICS

Marga Faulstich, Mainz, and Norbert Neuroth, Mainz-Mombach, Germany, assignors to JENAer Glaswerk Schott & Gen., Mainz, Germany

Filed June 22, 1970, Ser. No. 48,246

Claims priority, application Germany, June 25, 1969,

P 19 32 135.8

Int. Cl. C03c 3/04, 3/10; H03h 7/30

U.S. Cl. 106—53

9 Claims

#### ABSTRACT OF THE DISCLOSURE

Glass compositions for use in delay line assemblies having low temperature coefficient of propagation time for ultrasonic waves, low mechanical damping, a transformation temperature of about 540–600° C., and high acoustical impedance. Preferred compositions in percent by weight are as follows:

|                                      |           |
|--------------------------------------|-----------|
| SiO <sub>2</sub> -----               | 48.5–49.7 |
| Li <sub>2</sub> O -----              | 0–0.2     |
| Na <sub>2</sub> O -----              | 0–0.6     |
| K <sub>2</sub> O -----               | 0.7–1.0   |
| BaO -----                            | 10.5–11.5 |
| ZnO -----                            | 3.1–5.8   |
| PbO -----                            | 31–34     |
| Sb <sub>2</sub> O <sub>3</sub> ----- | 0.3–0.5   |

the total alkali metal oxide amounting to 0.7–1.8%, with the proviso that up to 2 of the wt. percent of BaO may be replaced by CdO, SrO, CaO, WO<sub>3</sub>, Al<sub>2</sub>O<sub>3</sub> or a mixture of two or more thereof, for stabilization against devitrification.

#### BACKGROUND

The invention relates to glasses for electromechanical delay lines which have a very low delay time temperature coefficient. Furthermore, these glasses have a relatively low mechanical damping, so that the intensity of the signal is only slightly attenuated by passing through the delay line.

In an electromechanical delay line, the electrical signal is transformed by a piezoelectric transducer into sound vibrations. These pass through the glass body and at the end of the sound path they are transformed back into electrical vibrations by a second piezoelectric transducer. The electrical signal at the output of the delay line is delayed by the amount of time which the sound takes to pass through the glass body. This travel time  $z$  is determined by the length  $L$  of the sound path and the velocity  $v$  of the sound in the glass, according to the equation  $z=L/v$ .

In a number of applications it is required that the temperature coefficient of time delay (T.C.) be very small, e.g.

$$\frac{1}{z} \frac{dz}{dT} = 2 \times 10^{-6} \text{ per } ^\circ \text{C.}$$

Our copending application Ser. No. 687,099, filed Dec. 1, 1967, now Pat. 3,615,770 is incorporated herein by reference; it explains the stated formula. With the glasses herein described it is possible to construct, for use with

## 2

piezoceramic transducers, delay lines which have a delay time temperature coefficient of this order of magnitude.

Two types of sound waves are possible in a solid: longitudinal waves and shear waves. In delay lines shear waves are preferred, because these waves have a lower velocity than longitudinal waves. The frequency, when measured, ranges around 5 megahertz.

Two factors are important in the attenuation of the electrical signal in passing through the line:

- 10 (a) The mechanical vibration damping of the glass;  
(b) The intimate fastening together of transducer and glass.

#### THE INVENTION

15 The logarithmic decrement of the mechanical vibration damping (L.D.) in the case of the glasses described in this invention, at a frequency of 1 kilohertz, amounts to  $0.35 \times 10^{-3}$  to  $0.45 \times 10^{-3}$ , that is, it is lower than it is in the special glasses of the prior art for this purpose. For example, in French Pat. No. 1,546,407 and copending application Ser. No. 687,099, filed Dec. 1, 1967, glasses are described in which  $\delta=2 \times 10^{-3}$  to  $5 \times 10^{-3}$ , and in German patent application p 16 96 064.8 and copending application Ser. No. 804,595, filed Mar. 5, 1969, glasses are described wherein  $\delta=0.5 \times 10^{-3}$  to  $0.8 \times 10^{-3}$ .

20 For (b) it is important that the glass be capable of good metallization. There are a number of processes for this purpose, e.g. vapor depositing and firing. For these processes it is desirable that the glass be able to withstand heating to high temperatures. The transformation temperature (T<sub>g</sub>) of the glasses of the invention just cited, ranges from 540 to 590° C.

25 The velocity of shear waves ( $v_s$ ) is lower in the glasses of the instant invention and the acoustical impedance (A.I.) is greater than in the case of the glasses hitherto described for temperature-stable ultrasonic delay lines which have a high softening temperature. Both of these factors represent technical improvements: the lower sound velocity signifies that the glass body can be made smaller, and the greater acoustical impedance means lower reflection losses in the passage of the sound waves from the glass to the transducer. The very low alkali oxide content in the glasses of the invention guards against mechanical after-effects.

30 35 40 45 The glasses of the invention have a small temperature coefficient of propagation time for ultrasonic waves, preferably for shear waves with a frequency of about 5 megahertz, with low mechanical dampening, transformation temperatures of about 540–600° C., and increased acoustical impedance. Preferred compositions are set forth in Table 2.

50 55 The total alkali metal oxide content amounts to 0.7 to 1.8%. For stabilization against devitrification, 2% of the BaO can be replaced by other alkali earth (SrO and CaO) or by CdO, WO<sub>3</sub>, or Al<sub>2</sub>O<sub>3</sub> without substantially modifying the special properties which are important to the described application of the glass.

#### BRIEF DESCRIPTION OF THE DRAWINGS

- 60 FIG. 1 is a schematic showing of a delay line assembly; and

65 FIG. 2 and FIG. 3 show change in delay time versus temperature for compositions of the invention stated infra.

Referring to FIG. 1, a delay line medium 1 is installed in an ultrasonic delay line assembly, which is of con-

ventional construction. The delay line medium is out-fitted with transducers 2 which are connected to input circuit 3 and output circuit 4.

#### Examples

In Table 1 there are listed a number of examples of glasses according to the invention. The chemical composition and the most important physical properties are stated:

TABLE 1

|                                                                 | 1     | 2     | 3     | 4     | 5     |
|-----------------------------------------------------------------|-------|-------|-------|-------|-------|
| Glass oxide:                                                    |       |       |       |       |       |
| SiO <sub>2</sub>                                                | 49.4  | 48.5  | 48.4  | 49.7  | 48.4  |
| Li <sub>2</sub> O                                               |       |       | 0.2   |       |       |
| Na <sub>2</sub> O                                               | 0.6   |       |       | 0.6   |       |
| K <sub>2</sub> O                                                | 0.7   | 1.0   | 0.3   | 0.7   | 1.0   |
| BaO                                                             | 11.2  | 10.5  | 11.5  | 11.1  | 11.5  |
| ZnO                                                             | 3.8   | 4.8   | 5.8   | 3.1   | 4.8   |
| PbO                                                             | 34.0  | 31.0  | 33.0  | 33.7  | 33.0  |
| Sb <sub>2</sub> O <sub>3</sub>                                  | 0.3   | 0.3   | 0.3   | 0.3   | 0.3   |
| CdO                                                             |       | 2.0   |       |       |       |
| WO <sub>3</sub>                                                 |       |       | 0.8   |       | 20    |
| Al <sub>2</sub> O <sub>3</sub>                                  |       |       |       | 1.0   |       |
| T.C.:                                                           |       |       |       |       |       |
| $\frac{1}{2} \frac{dz}{dT} \times 10^{-6}$ C. (10 . . . 60° C.) |       |       |       |       |       |
| 4.4 MHz.)                                                       | 1.2   | 0.8   | 1.5   | 1.2   | 1.2   |
| L.D. (log. decrement $\times 10^3$ )                            | 0.36  | 0.41  | 0.38  | 0.37  | 0.43  |
| (1 kHz.)                                                        |       |       |       |       | 25    |
| V <sub>s</sub> : Sound speed for shear waves, meters per sec.   | 2,722 | 2,733 | 2,742 | 2,727 | 2,730 |
| Density (g./cm. <sup>3</sup> )                                  | 3.58  | 3.58  | 3.63  | 3.57  | 3.59  |
| A.I.: Acoustical impedance, $10^6$ kg./m. <sup>2</sup> × sec.)  | 9.75  | 9.76  | 9.96  | 9.74  | 9.80  |
| Tg: Transformation temperature (° C.)                           | 550   | 572   | 555   | 542   | 577   |
|                                                                 |       |       |       |       | 30    |

As can be seen from Table 1, the compositional ranges of the glasses of the examples consist essentially of:

|                                |           |    |  |  |  |
|--------------------------------|-----------|----|--|--|--|
| SiO <sub>2</sub>               | 48.4-49.7 |    |  |  |  |
| Li <sub>2</sub> O              | 0-0.2     | 35 |  |  |  |
| Na <sub>2</sub> O              | 0-0.6     |    |  |  |  |
| K <sub>2</sub> O               | 0.3-1.0   |    |  |  |  |
| BaO                            | 10.5-11.5 |    |  |  |  |
| ZnO                            | 3.1-5.8   |    |  |  |  |
| PbO                            | 31.0-34.0 | 40 |  |  |  |
| Sb <sub>2</sub> O <sub>3</sub> | 0.3       |    |  |  |  |
| CdO                            | 0-2.0     |    |  |  |  |
| WO <sub>3</sub>                | 0-0.8     |    |  |  |  |
| Al <sub>2</sub> O <sub>3</sub> | 0-1.0     |    |  |  |  |

These glasses also have the following properties:

Temperature coefficient, 10 to 60° C. at 4.4 MHz., 0.8 to  $1.5 \times 10^{-6}$  per ° C.; mechanical damping in terms of logarithmic decrement at 1 kilohertz of about  $0.36 \times 10^{-3}$  to  $0.43 \times 10^{-3}$ ; sound speed for shear waves of 2722 to 2742 meters per second; density of 3.57 to 3.63 grams/cm.<sup>3</sup>; acoustical impedance of  $9.74$  to  $9.96 \times 10^6$  kg./m.<sup>2</sup> × sec.); and a transformation temperature in the range of about 550 to 577° C.

FIGS. 2 and 3 show the effect of temperature on the delay time in a delay line made from the glasses in the table and providing a 64 microsecond delay.

#### Production example

The glasses of the invention are similar in type to known optical and art glasses, and they can be produced by procedures which are conventional for production of such glasses. In the instant example, the batch mixture consists of:

| Oxide                          | Per-<br>cent<br>by wt. | Raw material                      | Amount<br>weighed<br>in, in kg.,<br>100 kg.<br>of glass |
|--------------------------------|------------------------|-----------------------------------|---------------------------------------------------------|
| SiO <sub>2</sub>               | 49.5                   | SiO <sub>2</sub>                  | 49.599                                                  |
| K <sub>2</sub> O               | 1.0                    | K <sub>2</sub> CO <sub>3</sub>    | 1.471                                                   |
| BaO                            | 5.1                    | Ba(NO <sub>3</sub> ) <sub>2</sub> | 8.726                                                   |
| BaO                            | 5.6                    | BaCO <sub>3</sub>                 | 7.263                                                   |
| ZnO                            | 4.9                    | ZnO                               | 4.907                                                   |
| CdO                            | 2.0                    | CdO                               | 2.007                                                   |
| PbO                            | 31.6                   | PbO                               | 32.362                                                  |
| Sb <sub>2</sub> O <sub>3</sub> | 0.3                    | Sb <sub>2</sub> O <sub>3</sub>    | 0.301                                                   |

The well-mixed batch is continuously fed into a conventional glass melting tank, melted at about 1440° C. in about 16 hours, refined for about 14 hours, at about 1480-1500° C. and until it is free of bubbles, and, at a viscosity between 300 and 500 poises (corresponding to temperatures of 1420 to 1360° C.), depending on the throughput, it is poured off and worked directly into the desired molded objects or bars. In this example, the viscosity at pouring off is about 6,000 poises. The melt can also be cast in blocks from which the desired objects can afterwards be pressed. The molded objects are annealed in accordance with conventional optical glass practice. The glass can also be produced in any smaller volume desired in platinum crucibles or appropriate ceramic crucibles.

A summary of the invention is contained in Table 2.

TABLE 2

|                                | Preferred<br>range | Optimum<br>range |
|--------------------------------|--------------------|------------------|
| Weight percent:                |                    |                  |
| SiO <sub>2</sub>               | 48.5-49.7          | 48.5-49.5        |
| Li <sub>2</sub> O              | 0-0.2              | 0                |
| Na <sub>2</sub> O              | 0-0.6              | 0-0.6            |
| K <sub>2</sub> O               | 0.7-1.0            | 0.7-1.0          |
| BaO                            | 10.5-11.5          | 10.5-11.5        |
| ZnO                            | 3.1-5.8            | 3.1-4.8          |
| PbO                            | 31-34              | 31-34            |
| Sb <sub>2</sub> O <sub>3</sub> | 0.8-0.5            | 0.3              |
| StO                            |                    |                  |
| CaO                            |                    |                  |
| CdO                            |                    |                  |
| WO <sub>3</sub>                |                    |                  |
| Al <sub>2</sub> O <sub>3</sub> |                    | 0-2 of the BaO   |
| T.C. <sup>1</sup>              | 0.8-1.5            | 0.8-1.2          |
| L.D. <sup>1</sup>              | 0.36-0.43          | 0.36-0.43        |
| V <sub>s</sub> <sup>1</sup>    | 2,720-2,745        | 2,722-2,742      |
| Density <sup>1</sup>           | 3.58-3.63          | 3.58-3.63        |
| A.I. <sup>1</sup>              | 9.74-9.96          | 9.74-9.96        |
| Tg <sup>1</sup>                | 550-577            | 550-577          |

<sup>1</sup> Units as in Table 1.

#### What is claimed is:

1. Glass having a low temperature coefficient of the propagation time for ultrasonic waves, mechanical damping in terms of logarithmic decrement at 1 kilohertz of about  $0.36 \times 10^{-3}$  to  $0.43 \times 10^{-3}$ , a transformation temperature in the range of about 550-577° C. and high acoustical impedance, consisting essentially of the following chemical composition in percent by weight:

|                                |           |    |  |
|--------------------------------|-----------|----|--|
| SiO <sub>2</sub>               | 48.4-49.7 |    |  |
| Li <sub>2</sub> O              | 0-0.2     |    |  |
| Na <sub>2</sub> O              | 0-0.6     |    |  |
| K <sub>2</sub> O               | 0.3-1.0   |    |  |
| BaO                            | 10.5-11.5 |    |  |
| ZnO                            | 3.1-5.8   |    |  |
| PbO                            | 31.0-34.0 | 40 |  |
| Sb <sub>2</sub> O <sub>3</sub> | 0.3       |    |  |
| CdO                            | 0-2.0     |    |  |
| WO <sub>3</sub>                | 0-0.8     |    |  |
| Al <sub>2</sub> O <sub>3</sub> | 0-1.0     |    |  |

2. Glass according to claim 1, having the following properties:

temperature coefficient, 10 to 60° C. at 4.4 MHz, 0.8 to  $1.5 \times 10^{-6}$  per ° C.; sound speed for shear waves of 2722 to 2742 meters per second; density of 3.57 to 3.63 grams/cm.<sup>3</sup>; acoustical impedance of 9.74 to  $9.96 \times 10^6$  kg./m.<sup>2</sup> × sec.).

3. Glass according to claim 1, characterized by the following chemical composition in percent by weight:

|                                |      |  |     |
|--------------------------------|------|--|-----|
| SiO <sub>2</sub>               | 49.4 |  |     |
| Na <sub>2</sub> O              | 0.6  |  |     |
| K <sub>2</sub> O               | 0.7  |  |     |
| BaO                            | 11.2 |  |     |
| ZnO                            | 4.9  |  |     |
| CdO                            | 2.0  |  |     |
| PbO                            | 31.6 |  |     |
| Sb <sub>2</sub> O <sub>3</sub> | 0.3  |  |     |
|                                |      |  | 0.3 |

4. Glass according to claim 1, characterized by the following composition in percent by weight:

|                                |      |
|--------------------------------|------|
| SiO <sub>2</sub>               | 49.7 |
| Na <sub>2</sub> O              | 0.6  |
| K <sub>2</sub> O               | 0.7  |
| BaO                            | 11.1 |
| ZnO                            | 3.1  |
| PbO                            | 33.7 |
| Sb <sub>2</sub> O <sub>3</sub> | 0.3  |
| WO <sub>3</sub>                | 0.8  |

5. Glass according to claim 1, characterized by the following composition in percent by weight:

|                                |      |
|--------------------------------|------|
| SiO <sub>2</sub>               | 48.4 |
| K <sub>2</sub> O               | 1.0  |
| BaO                            | 11.5 |
| ZnO                            | 4.8  |
| PbO                            | 33.0 |
| Sb <sub>2</sub> O <sub>3</sub> | 0.3  |
| Al <sub>2</sub> O <sub>3</sub> | 1.0  |

6. Glass according to claim 1, characterized by the following composition in percent by weight:

|                                |      |
|--------------------------------|------|
| SiO <sub>2</sub>               | 48.5 |
| K <sub>2</sub> O               | 1.0  |
| BaO                            | 10.5 |
| ZnO                            | 4.8  |
| PbO                            | 31.0 |
| Sb <sub>2</sub> O <sub>3</sub> | 0.3  |
| CdO                            | 2.0  |

7. Glass according to claim 1, characterized by the following composition in percent by weight:

|                                |      |
|--------------------------------|------|
| SiO <sub>2</sub>               | 48.4 |
| Li <sub>2</sub> O              | 0.2  |
| K <sub>2</sub> O               | 0.3  |
| BaO                            | 11.5 |
| ZnO                            | 5.8  |
| PbO                            | 33.0 |
| Sb <sub>2</sub> O <sub>3</sub> | 0.3  |

8. Glass having a low temperature coefficient of the

propagation time for ultrasonic waves, mechanical damping in terms of logarithmic decrement at 1 kilohertz of about  $0.36 \times 10^{-3}$ – $0.43 \times 10^{-3}$ , a transformation temperature in the range of about 550–577° C. and high acoustical impedance, consisting essentially of the following chemical composition in percent by weight:

|                                |           |
|--------------------------------|-----------|
| SiO <sub>2</sub>               | 48.5–49.7 |
| Li <sub>2</sub> O              | 0.0–0.2   |
| Na <sub>2</sub> O              | 0.0–0.6   |
| K <sub>2</sub> O               | 0.7–1.0   |
| BaO                            | 10.5–11.5 |
| ZnO                            | 3.1–5.8   |
| PbO                            | 31–34     |
| Sb <sub>2</sub> O <sub>3</sub> | 0.3–0.5   |

with the proviso that up to 2 of the wt. percent of BaO may be replaced by CdO, SrO, CaO, WO<sub>3</sub>, Al<sub>2</sub>O<sub>3</sub> or a mixture of two or more thereof, for stabilization against devitrification.

9. Glass according to claim 8, having the following properties:

temperature coefficient, 10 to 60° C. at 4.4 MHz., 0.8 to  $1.5 \times 10^{-6}$  per ° C.; sound speed for shear waves of 2720 to 2745 meters per second; density of 3.58 to 3.63 grams/cm.<sup>3</sup>; acoustical impedance of 9.74 to  $9.96 \times 10^6$  kg./m.<sup>2</sup>×sec.).

#### References Cited

##### UNITED STATES PATENTS

2,762,713 9/1956 Davis et al. ----- 106—53

##### FOREIGN PATENTS

1,807,831 8/1969 Germany ----- 106—53  
1,118,422 7/1968 Great Britain ----- 106—53  
132,387 5/1949 Australia ----- 106—53

TOBIAS E. LEVOW, Primary Examiner

M. L. BELL, Assistant Examiner

U.S. Cl. X.R.

333—30

UNITED STATES PATENT OFFICE  
CERTIFICATE OF CORRECTION

Patent No. 3,687,697 Dated August 29, 1972

Inventor(s) Marga Faulstich et al.

It is certified that error appears in the above-identified patent and that said Letters Patent are hereby corrected as shown below:

Col. 3, line 75, change "b<sub>2</sub>O<sub>3</sub>" to -- Sb<sub>2</sub>O<sub>3</sub> --.

Signed and sealed this 9th day of January 1973.

(SEAL)

Attest:

EDWARD M. FLETCHER, JR.  
Attesting Officer

ROBERT GOTTSCHALK  
Commissioner of Patents